

Dec. 11, 1934.

W. H. CHARCH ET AL

1,983,520

LAMINATED MATERIAL

Filed April 22, 1931

Fig. 1.



Fig. 2.



Fig. 3.



Fig. 4.



Fig. 5.



Fig. 6.



William Hale Charch & Henry A. Fiegel INVENTORS

W. H. Charch

ATTORNEY

## UNITED STATES PATENT OFFICE

1,983,520

## LAMINATED MATERIAL

William Hale Charch, Buffalo, and Theron G. Finzel, Kenmore, N. Y., assignors to Du Pont Cellophane Company, Inc., New York, N. Y., a corporation of Delaware

Application April 22, 1931, Serial No. 531,959

27 Claims. (Cl. 154—46)

This invention relates to a laminated material and more particularly to laminating metal foils to moistureproof materials.

Recently, there has been developed a new type of moistureproof material which comprises a base, such as a sheet or film of regenerated cellulose, sheets or webs of paper, sheets or films of gelatin, sheets or films of cellulose derivatives, etc. combined, as by being impregnated and/or thinly coated on one or both sides, with a moistureproofing composition containing a minor portion of a wax. In one of its modifications, the moisture-proofing composition comprises a cellulose derivative, a gum or resin, a wax with or without a plasticizer. In another modification, the moisture-proofing composition comprises a synthetic resin and a wax while in a third form it comprises a drying oil and a wax with or without a gum or resin.

In addition to possessing the moistureproof characteristic above mentioned, this material is non-tacky and preferably also transparent and flexible. By virtue of these characteristics this material has attained extensive and widespread use as a wrapping material and is particularly employed when it is desired to display the material wrapped and maintain the product, especially one which is susceptible to gain or loss in moisture, in its original condition.

Certain articles have been and still are wrapped in metal foils. Metal foils in general, and specifically aluminum foil, are moistureproof, if they are in the perfect continuous state and are maintained in such condition. However, metal foils due to their mode of production usually possess pin holes and as a result thereof the moisture-proof effect is destroyed. Moreover, due to lack of flexibility, moderate flexing of the foil generally results in ruptures, tears or creases which also aid in destroying the moisture-proof property, if present.

While the lack of flexibility of metal foils is in many cases a limitation, for certain purposes it is an advantage. For example, a package of goods in which the component elements are separately removed and used one at a time requires a wrapping material which possesses sufficient rigidity, so that the remaining contents of the package can be kept in position by flexing the excess wrapping material over the open end. Metal foils admirably serve this purpose.

We have found that the desirable characteristics of metal foils can be retained and the material made moistureproof, irrespective of their mode of production and use by securing, uniting

or joining metal foils with the aid of a thermoplastic substance, such as a waxy material, to moistureproof materials of the type above mentioned.

It is therefore an object of this invention to provide a laminated material comprising a moistureproof material of the type previously mentioned secured and united as by a thermoplastic substance, for example, a waxy material to metal foil.

Another object of this invention is to provide a method of securing, uniting, joining or laminating metal foils to moistureproof materials, such as moistureproof sheets or films of regenerated cellulose.

A further object of this invention is to provide a method of securing, joining, uniting or laminating metal foils to moistureproof materials, and particularly moistureproof sheets or films of regenerated cellulose, which comprises applying a thermoplastic substance, such as waxy materials in the fused state, to either one or both of the opposing surfaces of the materials, disposing the materials in superposed relationship and then causing the thermoplastic material to set.

Other objects will appear from the following description, appended claims and accompanying drawing forming a part of this specification and in which:

Figure 1 designates an enlarged cross-section of the material produced according to this invention.

Figure 2 diagrammatically illustrates one modification of a method constituting this invention.

Figure 3 illustrates an enlarged cross-section of a modification of the material illustrated in Figure 1.

Figure 4 illustrates another enlarged cross-section of a modification of the material illustrated in Figure 1.

Figures 5 and 6 illustrate enlarged cross-sections of two additional modifications.

Referring to the drawing in which like reference numerals designate like parts, and particularly Figure 1, the reference numeral 1 designates a metal foil, such as commonly used for wrapping materials, secured or laminated to a moistureproof material 2 through the medium of an adhesive-functioning material 3.

The lamina 2 may consist of any suitable base as, for example, a sheet or web of paper, a sheet or film of gelatin, a sheet or film of a cellulose derivative, such as a sheet or film of cellulose acetate, and preferably a sheet or film of regenerated cellulose, combined with a moisture-proofing

composition containing a minor proportion of a waxy composition. In the preferred form the base is coated and/or impregnated with a composition comprising a cellulose derivative, a resin and a wax with or without a plasticizer. In another modification, the base may be coated and/or impregnated with a composition comprising as the essential ingredients a synthetic resin and a wax, while in a third form the base may be coated and/or impregnated with a composition comprising a drying oil and a wax with or without a gum or resin.

The adhesive-functioning material 3 is a thermoplastic substance which is capable of softening under heat and of recovering its original characteristics on cooling. Preferably, also, the thermoplastic material is of such a nature that, after application and setting, it does not become hard and brittle.

As examples of thermoplastic materials which have been satisfactorily employed for securing the two materials together may be mentioned waxes, such as paraffin, beeswax, ceresin, or synthetic wax-like materials, such as hydrogenated oils, either alone or in combination with other waxy materials, such as wool grease, petroleum jelly, etc.

Referring to Figure 2 wherein one form of laminating the materials in accordance with the invention is diagrammatically illustrated, the thermoplastic materials 3, such as paraffin wax having a melting point of about 135° to 140° F., is disposed in a heated jacketed receptacle 4 where it is melted. In the fused condition the wax is applied to one surface of a moistureproof material 2 supplied from any suitable source, such as a roll 5 running, partly submerged, in the fused paraffin. The roll 5 may be provided with a suitable doctor blade (not shown) to regulate the quantity of wax applied. Alternatively, the excess of the wax may be removed from the moistureproof material in any suitable manner, such as by squeegees or doctor knives (not shown).

After the desired amount of wax has been applied to the moistureproof material, the foil withdrawn from the roll 6 is positioned on the coated face of the moistureproof material. The two materials are then passed through any suitable pressure means, such as calender rolls 7, preferably heated, and finally wound by any suitable winding mechanism into a roll 8. The material on the roll may be subsequently slit or fabricated as desired.

The distance between the pressure means 7 and the winding mechanism forming the roll 8 is such that the thermoplastic material is permitted to cool and set prior to winding. If desired, auxiliary cooling means, such as nozzles 9, spraying a cold medium, for example chilled air, on one or both sides of the material may be used to expedite the setting of the thermoplastic substance. The setting may also be effectively accomplished by passing the laminated material over one or more suitably chilled rolls as, for example, hollow rolls through which a cooling medium, such as brine or water, circulates.

It is, of course, apparent that instead of applying the thermoplastic material to the moistureproof sheet or film of regenerated cellulose, it may be applied to the metal foil or even to the opposing surfaces of both of the materials prior to the uniting thereof. It is also to be understood that means for applying the thermoplastic substance other than that specifically described

above may be employed. For instance, the fused thermoplastic substance may be applied by spraying or flowing it on the desired material.

Moistureproof sheets or films of regenerated cellulose are similar to non-moistureproof sheets or films of regenerated cellulose in that they are susceptible, although at an exceedingly low rate, to changes in the moisture content depending upon the atmospheric conditions in which they are disposed. Gain or loss of moisture is accompanied by swelling or shrinking respectively. Thus, when two sheets of material having different rates of swelling and shrinkage are laminated, there is a tendency for the product upon exposure to atmospheres of different humidities to wrinkle, curl or buckle in one way or the other depending upon the material which has the greater rate of change. Preshrunk sheets or films of regenerated cellulose, either of the coated or non-coated variety forming one or more plies in a laminated material, exhibit an appreciable resistance to curling, buckling or wrinkling, upon exposure to atmospheres of different humidities, such as atmospheres of relatively dry humidity.

When the moistureproof material 2 comprises a sheet or film of regenerated cellulose, the application of the hot fused wax thereto, prior to lamination, serves to preshrink the regenerated cellulose, whereby the extremely desirable properties of the preshrunk sheets are secured.

The product above mentioned, and which results from the method above explained, consists of metal foil laminated to a moistureproof material, such as a moistureproof sheet or film of regenerated cellulose, moistureproof paper, moistureproof sheet or film of gelatin or moistureproof sheet or film of a cellulose derivative, such as cellulose ester or ether. In other words, the foil is provided with a moistureproof sheet or film on one face thereof. It is, of course, apparent that various modifications of this form may be made and such modifications are contemplated by this invention. For instance, as illustrated in Figure 3, the foil 1 may be provided on both sides thereof with moistureproof materials, and the various laminae secured and united together through the medium of the thermoplastic substance 3. Similarly, as shown in Figure 4, the moistureproof sheet or film 2 may be sandwiched between two layers of metal foil 1. To produce these modifications the apparatus diagrammatically illustrated in Figure 2 may be modified so that the thermoplastic substance is applied to both sides of the material forming the inner ply of the product. Alternatively, the thermoplastic substance may be applied to the inner surfaces of the exterior plies and the inner ply led therebetween and finished as described.

The invention contemplates the lamination of sheets of foil and sheets of moistureproof materials of the same size by exactly superposing one on the other as described above and also by staggering one with respect to the other to produce a product as shown in Figure 5. It further contemplates the lamination of strips of foil in spaced relationship on a sheet of moistureproof material. For example, strips of foil 1 may be secured to a moistureproof sheet or film 2 as illustrated in Figure 6. If desired, the strips of foil 1 or the moistureproof material 2 may extend beyond the side edges of the other. In connection with the form of material illustrated in Figure 6, it is to be understood that the precise number of strips of material is not essential to

the successful practice of the invention, since any number may be used.

The appearance of the product may be materially enhanced by decorating, as by printing, painting, stippling, embossing or the like, the foil and/or employing variously colored or decorated moistureproof sheets or films of regenerated cellulose.

The above products are moistureproof to an exceedingly high degree and they may be used to wrap materials which are extremely sensitive to change in moisture content. The products, when viewed from the surface having the transparent, moistureproof sheet or film thereon, have a brilliant metallic luster. They also possess the desired rigidity of the foil. If for any reason the foil per se is or becomes non-moistureproof, it is of no material consequence. The moistureproof material secured thereto supplies the moistureproof characteristics to the product. This moistureproof property is retained even upon bending or flexing of the product. Thus, the product may be described as "permanently moistureproof".

To obtain optimum results, when the product is employed as a wrapper, it is desirable to effectively and securely seal the ends thereof. With this in view, the ends of the package may be dipped into molten wax to insure an effective closure. Similar results may be obtained by inserting in the ends of the package discs, preferably of any suitable material, such as paper-board impregnated with wax or the like, conforming to the cross-section of the package, and applying heat and preferably also pressure to the ends of said package. A very satisfactory seal between the end folds of the wrapper and the discs is thus obtained.

Since it is obvious that various modifications and changes may be made in the specific details described, this invention is not restricted thereto except as set forth in the appended claims.

We claim:

1. A flexible, non-greasy and substantially permanently moistureproof laminated wrapping material comprising a plurality of plies including a sheet or film of metal foil secured by a waxy substance to a moistureproof material consisting of a base coated on both sides thereof with a composition containing a minor proportion of wax.

2. A flexible, non-greasy and substantially permanently moistureproof laminated wrapping material comprising a plurality of plies including a sheet or film of metal foil secured by paraffin wax to a moistureproof material consisting of a base coated on both sides thereof with a composition containing a minor proportion of wax.

3. A flexible, non-greasy and substantially permanently moistureproof laminated wrapping material comprising a plurality of plies including a sheet or film of metal foil secured by a waxy substance to a transparent, moistureproof sheet or film of regenerated cellulose.

4. A flexible, non-greasy and substantially permanently moistureproof laminated wrapping material comprising a plurality of plies including a sheet or film of metal foil secured by paraffin wax to a transparent, moistureproof sheet or film of regenerated cellulose.

5. A flexible, non-greasy and substantially permanently moistureproof laminated wrapping material comprising a plurality of plies including a sheet or film of metal foil secured by a waxy substance to a moistureproof material consisting of

a base coated on both sides thereof with a composition comprising a cellulose derivative, a resin and a wax.

6. A flexible, non-greasy and substantially permanently moistureproof laminated wrapping material comprising a plurality of plies including a sheet or film of metal foil secured by paraffin wax to a moistureproof material consisting of a base coated on both sides thereof with a composition comprising a cellulose derivative, a resin and a wax.

7. A flexible, non-greasy and substantially permanently moistureproof laminated wrapping material comprising a plurality of plies including a sheet or film of metal foil secured by a waxy substance to a moistureproof material consisting of a base coated on both sides thereof with a composition comprising a cellulose derivative, a resin, a wax and a plasticizer.

8. A flexible, non-greasy and substantially permanently moistureproof laminated wrapping material comprising a plurality of plies including a sheet or film of metal foil secured by paraffin wax to a moistureproof material consisting of a base coated on both sides thereof with a composition comprising a cellulose derivative, a resin, a wax and a plasticizer.

9. A flexible, non-greasy and substantially permanently moistureproof laminated wrapping material comprising a plurality of plies including a sheet or film of metal foil secured by a waxy substance to a moistureproof material consisting of a sheet of paper coated on both sides thereof with a composition containing a minor proportion of wax.

10. A flexible, non-greasy and substantially permanently moistureproof laminated wrapping material comprising a plurality of plies including a sheet or film of metal foil secured by paraffin wax to a moistureproof material consisting of a sheet of paper coated on both sides thereof with a composition containing a minor proportion of wax.

11. A flexible, non-greasy and substantially permanently moistureproof laminated wrapping material comprising a plurality of plies including a sheet or film of metal foil secured by a waxy substance to a moistureproof material consisting of a sheet of paper coated on both sides thereof with a composition comprising a cellulose derivative, a resin and a wax.

12. A flexible, non-greasy and substantially permanently moistureproof laminated wrapping material comprising a plurality of plies including a sheet or film of metal foil secured by paraffin wax to a moistureproof material consisting of a sheet of paper coated on both sides thereof with a composition comprising a cellulose derivative, a resin and a wax.

13. A flexible, non-greasy and substantially permanently moistureproof laminated wrapping material comprising a plurality of plies including a sheet or film of metal foil secured by a waxy substance to a moistureproof material consisting of a sheet of paper coated on both sides thereof with a composition comprising a cellulose derivative, a resin, a wax and a plasticizer.

14. A flexible, non-greasy and substantially permanently moistureproof laminated wrapping material comprising a plurality of plies including a sheet or film of metal foil secured by paraffin wax to a moistureproof material consisting of a sheet of paper coated on both sides thereof with a composition comprising a cellulose derivative, a resin, a wax and a plasticizer.

15. A flexible, non-greasy and substantially permanently moistureproof laminated wrapping material comprising a plurality of plies including a sheet or film of metal foil secured by a waxy substance to a transparent, moistureproof material consisting of a sheet or film of regenerated cellulose coated on both sides thereof with a composition containing a minor proportion of wax.
16. A flexible, non-greasy and substantially 10 permanently moistureproof laminated wrapping material comprising a plurality of plies including a sheet or film of metal foil secured by paraffin wax to a transparent, moistureproof material consisting of a sheet or film of regenerated cellulose coated on both sides thereof with a composition 15 containing a minor proportion of wax.
17. A flexible, non-greasy and substantially 20 permanently moistureproof laminated wrapping material comprising a plurality of plies including a sheet or film of metal foil secured by a waxy substance to a transparent moistureproof material consisting of a sheet or film of regenerated cellulose coated on both sides thereof with a composition comprising a cellulose derivative, a resin and a wax.
18. A flexible, non-greasy and substantially 25 permanently moistureproof laminated wrapping material comprising a plurality of plies including a sheet or film of metal foil secured by paraffin wax to a transparent, moistureproof material consisting of a sheet or film of regenerated cellulose coated on both sides thereof with a composition comprising a cellulose derivative, a resin and a wax.
19. A flexible, non-greasy and substantially 30 permanently moistureproof laminated wrapping material comprising a plurality of plies including a sheet or film of metal foil secured by a waxy substance to a transparent, moistureproof material consisting of a sheet or film of regenerated cellulose coated on both sides thereof with a composition comprising a cellulose derivative, a resin, 35 and a wax.
20. A flexible, non-greasy and substantially 40 permanently moistureproof laminated wrapping material comprising a plurality of plies including a sheet or film of metal foil secured by paraffin wax to a transparent moistureproof material consisting of a sheet or film of regenerated cellulose coated on both sides thereof with a composition comprising a cellulose derivative, a resin, a wax and a plasticizer.
21. A flexible, non-greasy and substantially 45 permanently moistureproof laminated wrapping material comprising a plurality of plies including a sheet or film of metal foil secured by paraffin wax to a transparent moistureproof material consisting of a sheet or film of regenerated cellulose coated on both sides thereof with a composition comprising a cellulose derivative, a resin, a wax and a plasticizer.
22. A flexible, non-greasy and substantially 50 permanently moistureproof laminated wrapping material comprising a plurality of plies including a sheet or film of metal foil secured by paraffin wax to a transparent moistureproof sheet or film of regenerated cellulose, said sheet or film of regenerated cellulose being in a shrunken state.
23. A flexible, non-greasy and substantially 55 permanently moistureproof laminated wrapping material comprising a plurality of plies including a sheet or film of metal foil secured by paraffin wax to a transparent moistureproof material consisting of a sheet or film of regenerated cellulose coated on both sides thereof with a composition containing a minor proportion of wax, said sheet or film of regenerated cellulose being in the shrunken state.
24. A flexible, non-greasy and substantially 60 permanently moistureproof laminated wrapping material comprising a plurality of plies including a sheet or film of metal foil secured by paraffin wax to a transparent moistureproof material consisting of a sheet or film of regenerated cellulose coated on both sides thereof with a composition containing a minor proportion of wax, said sheet or film of regenerated cellulose being in the shrunken state.
25. A flexible, non-greasy and substantially 65 permanently moistureproof laminated wrapping material comprising a plurality of plies including a sheet or film of metal foil secured by paraffin wax to a transparent moistureproof material consisting of a sheet or film of regenerated cellulose coated on both sides thereof with a composition comprising a cellulose derivative, a resin and a wax, said sheet or film of regenerated cellulose being in the shrunken state.
26. A flexible, non-greasy and substantially 70 permanently moistureproof laminated wrapping material comprising a plurality of plies including a sheet or film of metal foil secured by a waxy substance to a transparent moistureproof material consisting of a sheet or film of regenerated cellulose coated on both sides thereof with a composition comprising a cellulose derivative, a resin, a wax and a plasticizer, said sheet or film of regenerated cellulose being in the shrunken state.
27. A flexible, non-greasy and substantially 75 permanently moistureproof laminated wrapping material comprising a plurality of plies including a sheet or film of metal foil secured by paraffin wax to a transparent, moistureproof material consisting of a sheet or film of regenerated cellulose coated on both sides thereof with a composition comprising a cellulose derivative, a resin, a wax and a plasticizer, said sheet or film of regenerated cellulose being in the shrunken state.

WILLIAM HALE CHARCH.  
THERON G. FINZEL.